

# UNITED STATES PATENT OFFICE.

CHRISTIAN ROSENTHAL, OF DETROIT, MICHIGAN.

## POLISH FOR VARNISHED SURFACES.

1,383,427.

Specification of Letters Patent.

Patented July 5, 1921.

No Drawing.

Application filed February 5, 1921. Serial No. 442,814.

*To all whom it may concern:*

Be it known that I, CHRISTIAN ROSENTHAL, a citizen of the United States of America, residing at Detroit, in the county 5 of Wayne and State of Michigan, have invented certain new and useful Improvements in Polish for Varnished Surfaces, of which the following is a specification.

The invention relates to polish for varnished surfaces and consists in the novel 10 composition as hereinafter set forth. My improved composition consists essentially of a wax, a solvent therefor, and amył acetate commercially known and referred to hereafter as banana oil. For the solvent I preferably employ gasolene, or an equivalent hydrocarbon oil, and I also add to the 15 banana oil an ingredient which will render the same miscible with this solvent, preferably a small quantity of oil of mirbane and 20 alcohol. I also preferably mix with the solvent a quantity of turpentine, as this increases the luster of the polish.

The specific formula which I preferably 25 use is as follows:

|                |        |
|----------------|--------|
| Wax            | 5 lb.  |
| Turpentine     | 10 lb. |
| Gasolene       | 10 lb. |
| Banana oil     | 4 lb.  |
| Oil of mirbane | 12 oz. |
| Alcohol        | 4 oz.  |

The method of compounding is; first, melt the wax and add the turpentine thereto. In 35 a separate vessel mix together the oil of

mirbane, alcohol and banana oil and then add to this mixture the gasolene. The two mixtures are then placed together and thoroughly commingled, with the result of forming a composition which is fluid at ordinary 40 temperatures.

In use, the mixture is spread over the surface, which is then polished by rubbing in the usual way.

What I claim as my invention is:

1. A polish comprising a wax, a solvent therefor, banana oil, and an ingredient for rendering said banana oil miscible with the solvent.

2. A polish comprising a wax, turpentine, 50 a mineral oil, banana oil, and an ingredient for rendering the banana oil miscible with the mineral oil.

3. A polish comprising a wax, turpentine, gasolene, banana oil, and oil of mirbane.

4. A polish comprising a wax, turpentine, gasolene, banana oil, oil of mirbane and alcohol.

5. A polish comprising the following ingredients in substantially the proportions 60 specified:

|                |        |
|----------------|--------|
| Wax            | 5 lb.  |
| Turpentine     | 10 lb. |
| Gasolene       | 10 lb. |
| Banana oil     | 4 lb.  |
| Oil of mirbane | 12 oz. |
| Alcohol        | 4 oz.  |

In testimony whereof I affix my signature.

CHRISTIAN ROSENTHAL.